

# UNITED STATES PATENT OFFICE.

HENRY MEYERS, OF HYDE PARK, PENNSYLVANIA.

## IMPROVED CONCRETE PAVEMENT.

Specification forming part of Letters Patent No. 42,589, dated May 3, 1864.

*To all whom it may concern:*

Be it known that I, HENRY MEYERS, of Hyde Park, in the county of Luzerne and State of Pennsylvania, have invented a new and Improved Concrete Pavement; and I do hereby declare that the following is a full, clear, and exact description of the same.

This invention relates to a composition which is particularly applicable to sidewalks, cellar-floors, &c., and is mixed together of sawdust, pulverized clay, coal-ashes, sand, and coal-tar, and spread on a foundation prepared of iron slag, cinders, coarse gravel, or other indestructible material cemented together by coal-tar.

To enable others skilled in the art to make and use my invention, I will proceed to describe it.

In putting down a pavement I first prepare the foundation, about three inches thick, of iron slag, cinders, coarse gravel, or some other suitable indestructible material, which is rendered solid by rolling with a heavy roller or by stamping. I then sprinkle it over with coal-tar, in order that the superincumbent composition may firmly unite with it.

The composition consists of sawdust, one part; pulverized clay, two parts; coal-ashes, two parts; sand, three parts. These ingre-

dients are intimately mixed with each other, and with a sufficient quantity of coal-tar to make a stiff mortar, and this mixture I spread on the foundation about two inches thick, more or less, and finally I add a light covering of my composition in a dry state—that is, without being mixed with coal-tar. Finally, I roll or stamp the whole until it is sufficiently hard.

This composition, when properly prepared and applied, as above described, produces a pavement which is very durable and quite impervious to water. It is peculiarly applicable to sidewalks, cellar-floors, and to such places in general where a dry hard floor or covering is desired. It can be made cheap and with comparatively little labor, and it resists all changes of the weather.

What I claim as my invention, and desire to secure by Letters Patent, is—

A concrete pavement composed of the ingredients above specified, and mixed together in about the proportion set forth, in combination with the foundation prepared as described.

HENRY MEYERS.

Witnesses:

T. J. LUCE,  
I. H. MILLSPAUGH.